# EUROPEAN PATENT SPECIFICATION

(11) **EP 0 029 523 B1**
(45) Date of publication and mention of the grant of the patent: **05.10.1983**
(21) Application number: 80106716.6
(22) Date of filing: 31.10.1980
(51) Int. Cl.: F21K 5/02

(54) **Miniature photoflash lamp and method of making**
Miniatur-Fotoblitzlampe und Verfahren zur Herstellung
Lampe-éclair photographique miniature et procédé de fabrication

(30) Priority: 21.11.1979 US 96606
(43) Date of publication of application: 03.06.1981
(73) Proprietor: GTE Products Corporation, Wilmington, DE 19801 (US)
(72) Inventor: Bouchard, Andre C., Peabody, Mass. 01960 (US)
(74) Representative: Lemke, Jörg-Michael, Dipl.-Ing.

## Description

The invention relates to photoflash lamps and particularly to photoflash lamps of the miniature variety (those having an internal volume of about 1.0 cubic centimeter or less), and to a method for making such lamps.

From US-A-3 220 224 there is known an electrically activated photoflash lamp comprising a light-transmitting envelope, a flash-producing composition located within said envelope for burning in a substantially localized manner to provide a flash of light, upon ignition thereof, said composition including a predetermined quantity of a powdered metal material and a predetermined quantity of a powdered oxidizer material, and means for electrically igniting said flash-producing composition, comprising a pair of conductive lead-in wires secured within a wall or end portion of said envelope and having exposed, conductive end portions extending within said envelope. In this prior art lamp the flash producing mixture is substantially physically separated from the lamp igniter, the filament, and the metallic supports or lead-in conductors. This requirement necessitates use of a comparably large lamp envelope and therefore precludes the design of miniature flash lamps. In a miniature flash lamp there is simply not enough room for physically separating the flash producing mixture from the other components required to be located within the lamp envelope.

Miniature flash lamps per se are prior known. One type, as disclosed in US-A-3893798 typically includes a quantity of shredded, combustible foil, and a pressurized combustion-supporting atmosphere within the envelope. It is essential that the envelope is hermetically sealed in order to contain the atmosphere and assure operability of the lamp.

It is the object of this invention to simplify the assembly of photoflash lamps of the miniature variety. This goal can be achieved, according to the invention, by suitably modifying the prior art photoflash lamp comprising, among others, a flash-producing composition including powdered metal material and powdered oxidizer material if and when that prior art lamp is modified so that said envelope has an internal volume equal to or less than about 1 cubic centimeter and said igniting means extend within said envelope and in contact with said flash-producing composition, as is known per se in photoflash lamps containing a filamentary combustible metal and combustion supporting gas, that said powdered metal material has a particle size within the range of from 10 to 150 microns, and that said lead-in wires each include an insulative coating thereon and are twisted about each other.

When the powdered metal material has a particle size within the specified range, the flash producing characteristics become satisfactory in spite of the physical closeness, and simultaneously the igniting means may be made very sturdy for ease of assembly without occupying an unacceptably large portion of precious space within a miniature lamp. Earlier it has not been recognized that a very important difference between flash lamps including a combustion-supporting atmosphere on the one hand, and flash lamps including an oxidant in lieu of that, is to be found in that in the latter type of lamp it is not necessary to hermetically seal the lamp envelope. As soon as it is not necessary to hermetically seal the lamp envelope, it becomes acceptable that the envelope material will not completely adhere to the lead-in wire(s). If the requirement of complete adherence can be dispensed with, it becomes feasible to use a coating between the wire, and the envelope material even in a mass production environment. If the lead-in wires can be provided with a coating, to insulate them from each other, it is feasible to use twisted wires, which leads to a very sturdy construction for the igniting means for its size.

Features of various embodiments of the invention may be gathered from subclaims 2-9.

From DE-C-1254963 there is known a method for making a miniature, electrically- activated photoflash lamp, said method comprising: providing a tubular, light-transmitting member having first and second open ends, positioning a pair of conductive lead-in wires within said first of said open ends and sealing said first open end with said wires therein such that an end portion of each of said wires extends within said tubular member, positioning a quantity of flash-producing material within said second open end of said tubular member and in operative engagement with said extending end of said lead-in wires, and sealing said second open end of said tubular member to define a light-transmitting envelope, said envelope having an internal volume equal to or less than about one cubic centimetre. The flash lamps made by this method are ones having a pressurized, combustion-supporting atmosphere. This prior art method is according to the invention characterized in that an insulative coating is provided on said lead-in wires, and said wires are twisted about each other, both prior to sealing said wires within said first of said open ends of said light-transmitting member, and that said flash-producing material includes a predetermined quantity of a powdered metal material and a powdered oxidizer material for burning in a substantially localized manner to provide a flash of light upon ignition thereof, said powdered metal material having a particle size within the range of 10 microns to 150 microns, and that said flash-producing material is positioned in contact with said extending end of said lead-in wires.

This method may be improved by using the steps recited in claims 11 or 12.

### Brief description of the drawings

Fig. 1 is an elevational view, in section, of a miniature photoflash lamp in accordance with a preferred embodiment of the invention; and
Fig. 2 represents a flow diagram of the steps of producing a miniature photoflash lamp in accordance with the teachings of the invention.

### Best mode for carrying out the invention

For a better understanding of the present invention together with other and further objects, advantages and capabilities thereof, reference is made to the following disclosure and appended claims in connection with the above described drawings.

With particular reference to Fig. 1, a miniature photoflash lamp 10 is shown as including a light-transmitting envelope 13, a flash-producing composition 15 within envelope 13 for providing the light output for lamp 10 upon ignition thereof, and ignition means 17 for igniting composition 15 to provide said output. By the term miniature is meant a lamp having an envelope with an internal volume no greater than about 1.0 cubic centimeter. Envelope 13 is preferably cylindrical (tubular), and in one embodiment of the invention possessed an internal diameter of about 0.343 centimeters, an internal length of about 10.00 centimeters, and a wall thickness of about 0.127 centimeters. The preferred material for envelope 13 is plastic (polypropylene) which, having the above dimensions, results in the envelope being translucent. It is understood, of course, that other plastic materials and dimensional variations are possible, including those which provide a transparent vessel. It is also possible to use glass as the envelope material.

Flash-producing composition 15 comprises a predetermined quantity of a powdered metal (serving as the fuel) and a predetermined quantity of oxidizer (serving as the oxygen supplier). The preferred powdered metal material is zirconium while the preferred oxidizer material is potassium chlorate. Other acceptable oxidizers include potassium perchlorate and sodium chlorate while another acceptable metal is hafnium.

As described above, one of the primary features of the instant invention is the use of a relatively large particle size metal powder as a key ingredient of the powdered flash-producing composition (15). It was found that zirconium powders having particle sizes ranging from about 10 to about 150 microns could be successfully used to provide desired light outputs without sacrificing containment of the finished product's envelope. Improvements in color temperature were also attained using these particles, and it was possible to readily adjust flash duration times. It was also found that large fuel particles, when combined with the aforedescribed oxidizers and positioned within the above envelope, burned at higher temperatures, emitted more light per unit weight, caused less pressure build-up, burned in a more localized manner, and were considerably less hazardous to handle, than similar mixtures containing fuels having "finely divided" (e.g., 1.8 microns) particles. Obviously, the above features are deemed truly significant in the photoflash lamp field.

When using the above zirconium powder, it was preferred to use an oxidizer having a particle size within the range of about 70 to about 150 microns. It is understood, however, that smaller sizes (e.g., 10 microns) could be used without adversely affecting the benefits derived from the present invention. Several successful combinations of the above materials are provided below.

The utilization of a plastic envelope 13 is possible when above flash-producing combination 15 is employed due to the lack of need for a combustion-supporting atmosphere within the envelope. Accordingly, it is not necessary to hermetically seal envelope 13 as is required for lamps containing combustible foils and similar materials. For ease of manufacture, however, envelope 13 contains an atmosphere of air which in effect serves to support combustion. Permitting air to remain in the envelope during formation thereof eliminates the costly procedures of either extracting such atmosphere (e.g., to form a vacuum) or injecting same at high pressures, as typically required in known miniature lamps.

It was determined that the aforedefined fuels, when used in plastic vessel lamps, should radiate at color temperatures of at least 4000 degrees K. The finished lamps of the instant invention were all capable of attaining these desired levels. It was also possible to obtain light outputs approaching 500 lumen seconds and, by varying the fuel-oxidizer ratios, to vary the pulse (flash) duration of the output from about 5 to 30 milliseconds. Specifically, increasing the oxidizer content resulted in flash durations approaching the higher time values while excess fuel material produced short durations. Use of large particle fuels in an air-containing plastic envelope further permitted employment of large quantities of composition 15, in comparison to existing miniature lamps. For example, it was possible to successfully utilize flash-producing compositions weighing from about_{'}25 to about 35 milligrams in a 1.0 cubic centimeter envelope. Higher ratios (composition: envelope volume) are attainable when using smaller sized envelopes.

Ignition means 17 is shown in Fig. 1 as including a pair of conductive lead-in wires 19 and 21 each having an 0.03 centimeters diameter copper wire cover by a .005 centimeters insulative coating. Wires 19 and 21 are twisted about each other (about 4 turns per centimeter) into the configuration shown and sealed within a bottom (end) portion of envelope 13. Understandably, it is also possible to secure these members within one of the envelope's side walls or within the opposing, upper end. Exposed ends 23 of wires 19 and 21 extend within envelope 13 approximately 0.318 centimeters and include thereon a quantity of primer material 25. As shown, ends 23 are spacedly oriented with portions of primer 25 located therebetween. Application of ignition voltage across the protruding ends 27 of wires 19 and 21 by a suitable power source (e.g., a piezoelectric element) typically associated with many of today's cameras results in generation of a spark across ends 23 and instantaneous ignition of primer 25. A typical ignition voltage is about 3000 volts. The deflagrating primer 25 in turn ignites powdered composition 15. It is preferred that primer 25 be located within composition 15 or protrude slightly therefrom as illustrated in Fig. 1. It is possible to eliminate primer 25 in the present invention and directly ignite composition 15 using the spark generated between ends 23 of wires 19 and 21. In such an arrangement, ends 23 are thus defined as being in operative engagement with composition 15 (e.g., by being inserted therein). It is preferred, however, to utilize primer 25 in that less energy will be required to achieve ignition of lamp 10. One example of a primer material successfully used included about 78 percent zirconium powder, 16 percent potassium perchlorate, 4 percent Alon C, and 2 percent nitrocellulose. Another suitable example included 50 percent zirconium, 30 percent potassium perchlorate, 10 percent tungstic oxide, 4 percent Alon C, 4 percent glass beads, and 2 percent nitrocellulose. All of the above percentages are by weight of the mixture. Methyl cellulose acetate was used as a solvent in preparation of both of the defined primers. Application of primer to the ends 23 of wires 19 and 21 was achieved by dipping these ends into the liquid suspension and withdrawing slowly (e.g., 0.635 centimeters per second). The coated ends were than sealed within the end of envelope 13 as illustrated. Approximately 0.5 to 1.0 milligram of primer was utilized in lamp 10.

Although it has been shown and described to ignite composition 15 electrically, it is also within the scope of the invention to utilize percussively actuated means for this purpose. By way of example, a metal primer tube such as described in US-A-3,535,063 (Anderson et al) could be employed and project from the bottom end of envelope 13. Deformation of the tube would result in deflagration of the fulminating material therein up through the tube and ignition of composition 15 located within the envelope 13 in a similar manner to that depicted in Fig. 1. The teachings of US-A-3,535,063, are thus incorporated herein by reference.

The following represent several examples of miniature photoflash lamps made in accordance with the teachings of the invention. In all of these examples, the upper portion (approximately 9 centimeters of the envelope's length) of envelope 13 was optically darkened (masked) and the defined light output readings were taken from only the remaining "active" light-transmitting region of the envelope. It is understood from the above that composition 15 occupies this region and that the optically darkened portion thus represents an expansion chamber for gases generated during ignition. In summary, the "active" region emits a relatively large proportion of the lamp's total output due primarily to the beneficial results of using large grain size fuels which assure localized burning. Accordingly, the total light output of the invention will be greater than that indicated below wherein optical masking was used on envelope 13.

### Example I

Flash-producing composition: 15.9 milligrams zirconium powder (particle size: 15-20 microns) and 14.1 milligrams potassium chlorate powder (particle size: less than 74 microns)
Illumination: 240 lumen seconds
Pulse Duration: 5-7 milliseconds.
Color Temperature: about 4200 degrees K.
Containment: excellent.

### Example II

Flash-producing composition: 15.9 milligrams zirconium powder (particle size: 15-20 microns) and 14.1 milligrams potassium chlorate powder (particle size: 74-149 microns).
Illumination: 400 lumen seconds.
Pulse Duration: 10-12 milliseconds.
Color Temperature: about 4200 degrees K.
Containment: excellent.

### Example III

Flash-producing composition: 15.9 milligrams zirconium powder (particle size: 44-74 microns) and 14.1 milligrams potassium chlorate powder (particle size: 74-149 microns).
Illumination: 350 lumen seconds.
Pulse Duration: 20 milliseconds.
Color Temperature: about 4200 degrees K.
Containment: excellent.

### Example IV

Flash-producing composition: 15.9 milligrams zirconium powder (particle size: 44-74 microns) and 14.1 milligrams potassium chlorate powder (particle size: less than 74 microns).
Illumination: 450 lumen seconds.
Pulse Duration: 20 milliseconds.
Color Temperature: about 4200 degrees K.
Containment: excellent.

### Example V

Flash-producing composition: 15.9 milligrams zirconium power (particle size: 74-149 microns) and 14.1 milligrams potassium chlorate powder (particle size: less than 74 microns).
Illumination: 370 lumen seconds.
Pulse Duration: 30 milliseconds.
Color Temperature: about 4200 degrees K.
Containment: excellent

The aforedescribed dual wire electrical ignition means (including primer) was used to ignite the described flash-producing compositions. A piezoelectric element served as the requisite voltage source.

In addition to the above, examples were made wherein the zirconium powder had a particle size less than 10 microns (e.g., 3 microns). Ignition of the lamps resulted in rupture of the plastic envelope.

The above lamps were each produced by initially providing a piece of elongated, polypropylene tubing having opposed (first and second) open ends and the described internal diameter (0.343 centimeters). The dual-wired electrical ignition means 17, with the wires 19 and 21 twisted together and having primer 25 thereon, was inserted within a first open end of the tube and said end sealed. Sealing was achieved using a heated aluminum block having a recessed (concave) portion with an aperture centrally located therein and passing through the block. Wires 19 and 21 were oriented within the block's aperture to extend within the recessed portion whereupon the polypropylene tubing was lowered about the wiring until engagement was effected between the recess and the tube's first open end. A small force was then exerted at the opposing, second open end of the tubing such that the first end was pressed against the block and deformed about the contained wiring. The tubing, now having ignition means 17 secured therein, was removed from the aluminum block and oriented vertically. The described quantity of flash-producing composition 15 was then dropped (using a funnel) into the upright tubing through the second open end. The composition fell to the bottom (first end) to surround the extending ends of wires 19 and 21 in the manner shown in Fig. 1. Positioning of composition 15 can be facilitated by moisture-dampening (e.g., using water) the composition prior to insertion. Such dampening resulted in a more homogeneous mixture (less particle segregation) than a simple dry (loose) mixture of the same material, particularly when using the larger, coarser grains. When dampening was used, the tubular members were located in an oven and dried (100 degrees C for about 10 minutes) prior to subsequent processing.

The next step in producing lamps 10 involved sealing the remaining (or second) open end. This process simply involved inserting the second end within the recess of the aforedescribed, heated aluminum block until closure was accomplished and a completed envelope was defined.

It is understood that the above process will result in. the surrounding atmosphere present during the last sealing step to become confined within the envelope, unless preventative steps (e.g. vacuum drawing) are taken. In a typical working environment, this atmosphere will obviously comprise air, an atmosphere totally satisfactory for permitting combustion of the invention's flash-producing composition therein.

This air will also be at normal atmospheric pressure when located therein and not at much higher pressures as typically required in known miniature lamps. Accordingly, the invention can be readily produced with less cost and difficulty than methods utilized in producing current_{'} miniature lamps which utilize combustible shred material. Furthermore, it is understood that envelope 13 needn't be completely (hermetically) sealed at either end as is required in the above, combustible-type lamps containing a pressurized, oxygen atmosphere therein.

## Claims

1. An electrically activated photoflash lamp comprising a light-transmitting envelope, a flash-producing composition located within said envelope for burning in a substantially localized manner to provide a flash of light, upon ignition thereof, said composition including a predetermined quantity of a powdered metal material and a predetermined quantity of a powdered oxidizer material, and means for electrically igniting said flash-producing composition, comprising a pair of conductive lead-in wires, secured within a wall or end portion of said envelope and having exposed, conductive end portions extending within said envelope, characterized in that said envelope has an internal volume equal to or less than about 1 cubic centimeter and said igniting means extend within said envelope and is in contact with said flash-producing composition, as is known per se in photoflash lamps containing a filamentary combustible metal and combustion supporting gas, that said powdered metal material has a particle size within the range of from 10 to 150 microns, and that said lead-in wires each include an insulative coating thereon and are twisted about each other.

2. The photoflash lamp according to claim 1 wherein the material for said envelope is selected from the group consisting of glass and plastic.

3. The photoflash lamp according to claim 2 wherein said plastic is polypropylene.

4. The photoflash lamp according to claim 1 wherein said powdered metal material is selected from the group consisting of zirconium and hafnium.

5. The photoflash lamp according to claim 1 wherein said powdered oxidizer is selected from the group consisting of potassium chlorate, potassium perchlorate, and sodium chlorate.

6. The photoflash lamp according to claim 1 wherein the ratio of said flash-producing composition to the internal volume of said envelope is within the range of 25 milligrams per cubic centimetre to 35 milligrams per cubic centimetre.

7. The photoflash lamp according to claim 1 wherein said powdered oxidizer material has a particle size within the range of from 70 microns to 150 microns.

8. The photoflash lamp according to claim 1 further including a combustion-supporting atmosphere within said envelope, said atmosphere comprised of air.

9. The photoflash lamp according to claim 1 further including a quantity of primer material positioned on said exposed, conductive end portions of said lead-in wires and in contact with said flash-producing composition for igniting said composition, said conductive end portions and said primer material positioned substantially within said flash-producing composition.

10. A method of making a miniature, electrically-activated photoflash lamp, said method comprising: providing a tubular, light-transmitting member having first and second open ends, positioning a pair of conductive lead-in wires within said first of said open ends and sealing said first open end with said wires therein such that an end portion of each of said wires extends within said tubular member, positioning a quantity of flash-producing material within said second open end of said tubular member and in operative engagement with said extending end of said lead-in wires, and sealing said second open end of said tubular member to define a light-transmitting envelope, said envelope having an internal volume equal to or less than about one cubic centimetre, characterized in that an insulative coating is provided on said lead-in wires, and said wires are twisted about each other, both prior to sealing said wires within said first of said open ends of said light-transmitting member, and that said flash-producing material includes a predetermined quantity of a powdered metal material and a powdered oxidizer material for burning in a substantially localized manner to provide a flash of light upon ignition thereof, said powdered metal material having a particle size within the range of 10 microns to 150 microns, and that said flash-producing material is positioned in contact with said extending end of said lead-in wires.

11. The method according to claim 10 further including providing a quantity of primer material on said extending ends of said lead-in wires prior to positioning said flash-producing composition within said tubular member.

12. The method according to claim 10 further including adding a combustion-supporting atmosphere within said tubular member through said second end of said tubular member immediately prior to sealing said second end.

## Patentansprüche

1. Elektrisch aktivierte Photoblitzlampe bestehend aus einem lichtdurchlässigen Kolben, einer blitzerzeugenden Mischung, die im Kolben angeordnet ist, um in einer im wesentlichen lokalisierten Weise nach Zündung so zu verbrennen, daß ein Lichtblitz geliefert wird, wobei diese Mischung eine vorbestimmte Menge eines pulverförmigen metallischen Werkstoffes und eine vorgegebene Menge eines gepulverten Oxydationsmaterials enthält, und Mitteln zum elektrischen Zünden der blitzerzeugenden Mischung, bestehend aus einem Paar leitender Zulietungsdrähte, die in einer Wand oder einem Endteil des Kolbens festgelegt sind und freigelegte, lietende Endteile aufweisen, die sich in den Kolben hinein erstrecken, dadurch gekennzeichnet, daß der Kolben ein Innenvolumen gleich oder kleiner als etwa 1 Kubikzentimeter hat und die Zündmittel sich in den Kolben hinein erstrecken und in Kontakt mit der blitzerzeugenden Mischung stehen, wie an sich in Photobilitzlampen bekannt die ein verbrennbares Metall in Fadenform und ein verbrennungsförderndes Gas enthalten, daß der pulverförmige metallische Werkstoff eine Partikelgröße im Bereich von 10-150 Mikron hat, und daß die Zuleitungsdrähte jeweils eine isolierende Beschichtung tragen und umeinander verdrillt sind.

3. Photoblitzlampe nach Anspruch 1 bei der Werkstoff für den Kolben aus der Gruppe gewählt ist, die aus Glas und Kunststoff besteht.

3. Photoblitzlampe nach Anspruch 2, bei der der Kunststoff Polypropylen ist.

4. Photoblitzlampe nach Anspruch 1 bei der der pulverförmig metallische Werkstoff aus der Gruppe ausgewählt ist, die aus Zirkon und Hafnium besteht.

5. Photoblitzlampe nach Anspruch 1 bei der das gepulverte Oxydationsmittel aus der Gruppe ausgewählt ist, die aus Kaliumchlorat, Kaliumperchlorat und Natriumchlorat besteht.

6. Photoblitzlampe nach Anspruch 1 bei der das Verhältnis der blitzerzeugenden Mischung zum Innenvolumen des Kolbens im Bereich von 25 Milligramm pro Kubikzentimeter bis 35 Milligram pro Kubikzentimeter liegt.

7. Photoblitzlampe nach Anspruch 1 bei der der pulverförmige Oxydationsmittel-Werkstoff eine Partikelgröße im Bereich von 70 Mikron bis 150 Mikron hat.

8. Photoblitzlampe nach Anspruch 1, die weiter eine verbrennungsfördernde Atmosphäre innerhalb des Kolbens aufweist, wobei diese Atmosphäre aus Luft besteht.

9. Photoblitzlampe nach Anspruch 1, die weiter eine Menge eines Zünderwerkstoffes aufweist, die auf den freigelegten, leitenden Endteilen der Zuleitungsdrähte angeordnet ist, und in Berührung mit der blitzerzeugenden Mischung, zur Zündung der Mischung, wobei die leitenden Enden und der Zünderwerkstoff im wesentlichen innerhalb der blitzerzeugenden Mischung positioniert sind.

10. Verfahren zur Herstellung einer elektrisch betätigten Miniatur-Photoblitzlampe, bestehend aus der Schaffung eines rohrförmigen, lichtdurchlässigen Elementes mit ersten und zweiten offenen Enden, dem Positionieren eines Paares von leitenden Zuleitungsdrähten in das erste der offenen Enden und Verschließen des ersten offenen Endes mit den darin befindlichen Drähten derart, daß ein Endteil der Drähte sich in das rohrförmige Element hinein erstreckt, Positionieren einer Menge eines blitzerzeugenden Werkstoffes in das zweite offene Ende des rohrförmigen Elementes und in betrieblichen Eingriff mit dem vorstehenden Ende der Zuleitungsdrähte, und Verschließen des zweiten offenen Endes des rohrförmigen Elements um einen lichtdurchlässigen Kolben zu bilden, wobei dieser Kolben eine Innenvolumen gleich oder kleiner als etwa 1 Kubikzentimeter hat, dadurch gekennzeichnet, daß eine isolierende Schicht auf den Zuleitungsdrähten vorgesehen wird und die Drähte umeinander verdrillt werden, beides vor dem Einsiegeln der Drähte in das erste der offenen Enden des lichtdurchlässigen Elementes, und daß das blitzerzeugende Material eine vorgegebene Menge eines pulverförmigen metallischen Werkstoffs und eines pulverförmigen Oxydationsmittel-Werkstoffes enthält, um nach Zündung in einer im wesentlichen lokalisierten Weise zu verbrennen, um nach seiner Zündung einen Lichtblitz zu erzeugen, wobei der pulverförmige metallische Werkstoff eine Partikelgröße im Bereich von 10 Mikron bis 150 Mikron hat, und daß das blitzerzeugende Material in Kontakt mit dem vorstehenden Ende der Zulietungsdrähte positioniert wird.

11. Verfahren nach Anspruch 10, das weiter einschließt das Aufbringen einer Menge eines Zünderwerkstoffes auf die vorstehenden Enden der Zuleitungsdrähte vor dem Positionieren der blitzerzeugenden Mischung in das rohrförmige Element.

12. Verfahren nach Anspruch 10, das weiter einschließt die Hinzufügung einer verbrennungsfördernden Amosphäre innerhalb des rohrförmigen Elementes durch das zweite Ende des rohrförmigen Elementes unmittelbar vor dem dichten Verschließen dieses zweiten Endes.

## Revendications

1. Lampe à éclair à usage photographique, à commande électrique, comprenant une ampoule transparente, et à l'intérieur de celle-ci, une composition produisant l'éclair devant brûler de manière pratiquement localisée et délivrer un éclair, après mise en ignition, la dite composition incluant une quantité déterminée d'un matériau métallique en poudre et une quantité determinée d'un matériau oxydant en poudre, ainsi que des moyens pour commander électriquement la mise en ignition de la composition produisant l'éclair, incluant deux entrées de courant, fixées dans le pied de la dite ampoule et dont les extrémités conductrices visibles font saillie à l'intérieur de l'ampoule, caractérisée en ce que le volume interne de la dite ampoule est inférieur ou égal à un centimère cube et que les dits moyens pour commander la mise en ignition font saillie à l'intérieur de la dite ampoule et sont en contact avec la dite composition produisant l'éclair, comme il est connu en soi dans les lampes à éclair contenant un métal combustible sous forme de clinquants et un gaz favorisant la combustion, que le diamètre des particules constituant le dit matériau métallique en poudre est compris entre 10 et 150 microns, et que les dites entrées de courant sont recouvertes chacune d'un revêtement isolant et sont tressées.

2. Lampe à éclair selon la revendication 1, caractérisée en ce que le matériau constituant la dite ampoule est choisi dans le groupe comprenant le verre et le plastique.

3. Lampe à éclair selon la revendication 2, caractérisée en ce que le dit plastique est du polypropylène.

4. Lampe à éclair selon la revendication 1, caractérisée en ce que le dit matériau métallique en poudre est choisi dans le groupe comprenant le zirconium et l'hafnium.

5. Lampe à éclair selon la revendication 1, caractérisée en ce que le dit oxydant en poudre est choisi dans le groupe comprenant le chlorate de potassium, le perchlorate de potassium et le chlorate de sodium.

6. Lampe à éclair selon la revendication 1, caractérisée en ce que le poids de la composition produisant l'éclair par rapport au volume interne de la dite ampoule est compris entre 25 et 35 mg/cm³.

7. Lampe à éclair selon la revendication 1, caractérisé en ce que le diamètre des particules du matériau oxydant en poudre est compris entre 70 et 150 microns.

8. Lampe à éclair selon la revendication 1, caractérisée en ce que la dite ampoule comprend un gaz favorisant la combustion, le dit gaz incluant de l'air.

9. Lampe à éclair selon la revendication 1, caractérisée en ce qu'une quantité de matériau d'amorçage est disposé sur l'extrémité interne conductrice et visible des dites entrées de courant et en contact avec la dite composition produisant l'éclair pour en permettre la mise en ignition, les dites extrémités internes conductrices et le dit matériau d'amorçage étant disposés pratiquement à l'intérieur de la composition produisant l'éclair.

10. Procédé de fabrication d'une lampe à éclair miniature à usage photographique, à commande électrique, comprenant les étapes suivantes:
- on dispose un tube transparent ayant une première et une seconde extrémités ouvertes,
- on met en place deux entrées de courant conductrices par la première entrée ouverte,
- on scelle la dite première extrémité ouverte avec les dites entrées de courant de telle manière qu'une extrémité de chacune des dites entrées fasse saillie à l'intérieur du dit tube,
- on introduit une quantité de matériau produisant l'éclair par la dite seconde extrémité ouverte du dit tube et la mettre en contact avec la partie faisant saillie des dites entrées,
- on scelle la dite seconde extrémité ouverte du dit tube pour déterminer une ampoule transparente, celle-ci présentant un volume interne inférieur ou égal à un centimètre cube environ, une ampoule transparente, celle-ci présentant un volume interne 15 le dit procédé étant caractérisé en ce qu'on dispose un revêtement isolant sur les dites entrées de courant, lesquelles sont tressées, avant de sceller les dites entrées dans la dite première extrémité ouverte du dit tube transparent, et que le dit matériau produisant l'éclair comprend une quantité déterminé d'un matériau métallique en poudre et d'un matériau oxydant en poudre pour brûler de manière substantiellement localisée pour délivrer un éclair après mise en ignition, le diamètre des particules du dit matériau métallique en poudre étant compris entre 10 et 150 microns, et que le matériau produisant l'éclair est mis en contact avec l'extrémité faisant sailie des dites entrées de courant.

11. Procédé selon la revendication 10, caractérisé en ce qu'on dispose une quantité de matériau d'amorçage sur les extrémités faisant saillie des dites entrées de courant avant d'introduire la composition produisant l'éclair à l'intérieur du dit tube.

12. Procédé selon la revendication 10, caractérisé en ce qu'on ajoute en outre un gaz favorisant la combustion à l'intérieur du dit tube par la dite seconde extrémité ouverte juste avant de sceller cette dernière.
